

# UNITED STATES PATENT OFFICE.

JAMES NICLES, OF SAN FRANCISCO, CALIFORNIA, ASSIGNOR OF ONE-THIRD TO  
WILLIAM G. WEISS, OF SAN FRANCISCO, CALIFORNIA.

## PAINT AND VARNISH REMOVER.

1,034,819.

Specification of Letters Patent. Patented Aug. 6, 1912.

No Drawing.

Application filed October 27, 1910. Serial No. 589,382.

*To all whom it may concern:*

Be it known that I, JAMES NICLES, a citizen of the United States of America, residing in the city and county of San Francisco 5 and State of California, have invented new and useful Improvements in Paint and Varnish Removers, of which the following is a specification.

The object of my invention is to produce 10 an improved paint and varnish remover which will perform its work in faster time than is possible with the present agencies of the kind, and which shall perform its work 15 is such a manner as to eliminate the need for going over with benzin the surface of the material from which the paint or varnish has been removed.

The largest part of the expense in operating paint removers is the labor; and my invention 20 consists in providing in a varnish and paint remover means for lessening the labor required at present.

It also consists in a paint and varnish remover of a fluid consistency, sufficiently 25 thickened to prevent its running unduly by some means which shall not dry.

It also consists in a paint and varnish remover that will remove paint and varnish without removing the stain or wood filling.

I cannot accomplish my object or produce 30 the desired results by the use of wax as a thickener for my fluid, because wax dries, and necessitates the washing of the surface from which the paint or varnish has been 35 removed with benzin or equivalent substance. But I do accomplish my object by the use of tallow as an ingredient of my paint and varnish remover. Tallow applied 40 as described below will thicken the fluid sufficiently and allow the coatings thereof to be wiped off without removing the filling or stain and without necessitating a further going over of the surface with benzin.

My paint and varnish remover consists of 45 acetone, by volume twenty-six per cent., denatured alcohol twenty-four and one-half per cent.; refined benzin seventeen per cent.;

ether three per cent.; tallow twenty per cent., powdered ammonium carbonate one and one-half per cent., and turpentine eight 50 per cent.

The ingredients are mixed as follows: The tallow is first boiled and drawn off; the alcohol and turpentine and ammonium carbonate are heated together, and the warm 55 tallow is added and shaken until thoroughly incorporated. The refined benzin, ether and acetone in a cold state are then mixed therewith, shaken for about ten minutes and the resulting mixtures strained. 60

In paint removers at present in use the principal active ingredient is wood alcohol. The fumes of wood alcohol are extremely injurious and for this reason I have adopted the combination of ether, ammonium carbonate, acetone and denatured alcohol, 65 which acts with the commercial efficiency of wood alcohol and without its injurious effects. The volatility of the substances last above referred to interfere with their activity for the purpose in view. But both the turpentine and the tallow tend to retard evaporation and therefore produce the desired result. 70

Having described my invention, what I 75 claim as new and desire to secure by Letters Patent of the United States is:

In a paint and varnish remover the combination with acetone, denatured alcohol, refined benzin, ether, ammonium carbonate, 80 and turpentine, of twenty per cent. of tallow mixed and combined substantially as described, whereby the after treatment of the surfaces by benzin would be rendered unnecessary. 85

In testimony whereof, I have hereunto subscribed my name, in the presence of two subscribing witnesses, in the city and county of San Francisco and State of California, this 27th day of August, in the year 1910. 90

JAMES NICLES.

In the presence of—

FRANK P. MEDINA,  
W.M. G. WEISS.